

# UNITED STATES PATENT OFFICE.

HERMANN GOETTER, OF NEW YORK, N. Y., ASSIGNOR TO THE ARLINGTON MANUFACTURING COMPANY, OF SAME PLACE AND ARLINGTON, NEW JERSEY.

## PYROXYLIN COMPOUND.

SPECIFICATION forming part of Letters Patent No. 597,144, dated January 11, 1898.

Application filed July 22, 1896. Serial No. 600,110. (No specimens.)

*To all whom it may concern:*

Be it known that I, HERMANN GOETTER, Ph. D., a subject of the Emperor of Germany, residing at New York, in the county of New 5 York and State of New York, have invented a new and useful Pyroxylin Compound to be Employed in the Arts and Trades, of which the following is a specification.

My invention has reference to an artificial 10 solid substance which is used for the same purposes as celluloid, pyralin, and similar compositions. The commercially-successful compositions of this kind consist, essentially, of nitrocellulose and camphor. The latter 15 makes these compositions very expensive, and it has been the aim of inventors to discover compositions free of camphor which answer the same purposes.

It is the special object of my invention to 20 produce a very cheap composition of this kind, and I have succeeded in producing a material in which the use of camphor is preferably entirely dispensed with.

My new composition, further, is easier 25 worked into articles, and the manufactured goods are superior in appearance and elasticity to those of similar materials.

My novel material is essentially composed 30 of nitrated cellulose and acetate of amyl.

In manufacturing the solid material I sub- 35 stantially proceed as follows: The nitrated cellulose is treated with an auxiliary solvent, preferably wood-alcohol or acetone or similar agents and acetate of amyl, simultaneously or in succession. After thus compounding the mass the wood-alcohol is mostly removed in a similar way as is usually employed in the manufacture of celluloid. For obtaining a first-class product it is important that the 40 nitrocellulose pulp is soft and fine. The mass so compounded is now subjected to rollers and manipulated by means of heat and pressure and seasoned in the usual manner. The proportions in which the single components 45 are employed may be varied.

For most purposes I prefer to use the following formula: twelve and one-eighth parts, by weight, of nitrocellulose, ten parts, by weight, of wood-alcohol, and three and one-half parts, 50 by weight, of acetate of amyl.

For certain articles of manufacture some

camphor may be mixed in. In such instances I prefer to use a composition of the following formula: twenty-four and one-fourth parts, by weight, of nitrocellulose, two parts, by 55 weight, of camphor, six parts, by weight, of acetate of amyl, and fifteen parts, by weight, of wood-alcohol. The proportions of this composition may also be varied.

If the pulp of the nitrocellulose is soft and 60 very fine, then the quantity of the wood-alcohol is reduced in proportion to the fineness and softness of the same. The use of acetate of amyl in the manufacture of such materials not only cheapens the final product, (the present 65 price of acetate of amyl is about one-fourth of the price of camphor,) but it also greatly facilitates the process of making them, because acetate of amyl is a solvent of nitrocellulose, and therefore a more transparent, 70 elastic, and beautiful product is obtained.

The solid finished material has naturally a slightly-yellowish tint of color. For certain articles the same may be colored in the usual manner. For less expensive articles so-called 75 "pigments" may be incorporated in order to increase the weight and to reduce the cost. Such pigments are, for instance, oxid of zinc, carbonate of magnesium, and similar substances. They are used either singly or mix- 80 tures thereof.

My novel invention further presents marked advantages over similar materials. When entirely free of camphor, then the obnoxious smell of camphor is certainly not 85 present, while the smell of acetate of amyl is not more perceptible after the seasoning of the mass. If ignited, it does not give off any bad odors and it does not smoke. The manufactured articles are very durable and of great 90 elasticity, an advantage which is, for instance, very valuable in combs manufactured therefrom. It further attains a high polish very easily.

I am aware of the fact that acetate of amyl 95 was known long ago as a solvent for nitrated cellulose and that, for instance, celluloid varnish is prepared with this solvent; but I claim that I have first discovered the specific compound described and the proportions specified for obtaining a solid commercial product. 100

Having now described my invention, what

I claim therein as new, and desire to secure by Letters Patent, is—

1. As a new article of manufacture, a solid composition to be used as a material in the arts and trades and composed essentially of about twelve parts by weight of nitrated cellulose and of about three and one-half parts by weight of acetate of amyl, as specified.

2. The process of manufacturing an artificial solid material consisting in compounding about twelve parts by weight of nitrated cellulose with an auxiliary solvent and about three and one-half parts by weight of acetate

of amyl, then removing nearly all the auxiliary solvent and the excess of the acetate of amyl and then manipulating the mass by heat and pressure to obtain the solid product, as specified.

In testimony whereof I have hereto set my hand in the presence of two subscribing witnesses.

HERMANN GOETTER.

Witnesses:

WILLIAM L. PERKINS,  
FRANK A. BUTLER.